

# UNITED STATES PATENT OFFICE.

JAMES MILN, OF TORONTO, ONTARIO, CANADA.

## COATED PAPER.

Patented May 7, 1918.

1,265,357.

No Drawing.

Specification of Letters Patent.

Application filed October 4, 1917. Serial No. 194,697.

To all whom it may concern:

Be it known that I, JAMES MILN, a subject of the King of Great Britain, residing at the city of Toronto, in the county of York 5 and Province of Ontario, Dominion of Canada, have invented certain new and useful Improvements in Coated Paper; and I hereby declare that the following is a full, clear, and exact description of the same.

10 The present invention relates to a coated paper which may be used in mechanical processes for the production of surfaces for printing illustrations when such surfaces are adapted to be attached to printing cylinders 15 or platens or to the lower surfaces of printing blocks in such a manner that the pressure to be exerted upon the different parts of the sheet to be printed upon is regulated according to the light and shade of the picture, 20 and the invention consists of applying to a paper surface a coating of etchable material, which, after the impression of the picture thereon with an etch-proof color, is subjected to an etching process, whereby the high 25 lights left uncovered or lightly covered by the color may be more or less deeply or completely etched by the action of the etching agent, and removed by washing or brushing.

30 Satisfactory results are obtainable by applying to the surface of the paper an etchable body capable of dissolution when subjected to the action of an etching agent, such 35 a body being preferably made by thoroughly mixing together in a dry state, blanc fixe, china clay, and an adhesive.

It is preferred to mix the blanc fixe and 40 china clay in the proportion of two hundred and ninety pounds of blanc fixe to five hundred and eighty pounds of china clay, free or substantially free from hard and gritty particles and substances, to which is added approximately sixty-five gallons of water, and then combining with the mixture a solution 45 consisting of approximately one hundred and twenty-five pounds of glue, twenty-five gallons of water, two pounds of glycerin and twelve ounces of aluminum acetate. The preferred solution which is employed 50 to effect the etching, is a 3° Baumé solution of bleaching powder, commonly called "chlorid of lime." This solution causes an etch on the coating, because of the fact that the hypochlorous acid in the solution readily destroys the binding quality of the thin

55 film of glue that binds the very minute particles of the inert materials used, and thereby allows these particles to be washed away. The etching solution has no action on the inert materials used, such as blanc fixe and 60 china clay. If water were used, the glue would merely be softened, with the result that the etch would be entirely unsuited for 65 the high class of work that is required from the paper.

The aluminum acetate used in the composition because of its acid reaction with the etching solution, liberates an excess of the active reagent from the etching solution during the process of etching, and thereby aids 70 as well as hastens the etch.

It is possible, however, to use instead of aluminum acetate, such reagents as ferrous sulfate, copper sulfate, copper chlorid, ferric chlorid, or other reagents having an acid 75 reaction, the acidity of which will tend to aid the etching qualities of the coating by liberating the excess of the active reagent from the etching solution.

It is preferred to use, in the preparation 80 of the solution, those grades of glue commercially known as "gelatin," having a high jelly strength, which are free or substantially free from chondrin, and it is preferred to soak the gelatin over night and then heat 85 it until in solution, when the glycerin and aluminum acetate are added, the solution being well stirred to intimately mix the ingredients.

Any appropriate color may be used to 90 part to the paper the required tint, and the coloring matter employed should be free from lumps. A preservative, such as a volatile oil, may be added to the glue solution. The mixture should be strained through 95 very fine sieves before using.

The aluminum acetate solution may be made by dissolving twelve ounces of lead acetate in two quarts of water and twelve ounces of aluminum sulfate in two quarts 100 of water, the two solutions being subsequently mixed together and permitted to stand. When the lead sulfate has settled out on the bottom, as much as possible of the solution may be poured out.

105 To prevent shrinkage in the paper after etching, the paper, before the coating is applied, should be washed to remove the original size, then resized with a solution of water and casein mixture, in the proportion

of three gallons of water to two quarts of casein mixture. The casein mixture should contain eight ounces of casein to one quart of solvent. After resizing, the paper should 5 be put through a weak acid solution, containing one and one-half ounces of concentrated hydrochloric acid to one gallon of water. This treatment applies to animal or glue sized papers. Casein and resin sized 10 papers do not need this treatment.

The paper when it has been coated with this etchable mass, is calendered or pressed between the calender rolls to produce a good printing surface, and is then ready for use 15 in the printing press, thereafter being subjected to the etching process.

The etching process consists of the application of an etch-proof color either on one side of the coated paper or on both sides, to 20 increase the effect; in which latter case, the printing block, with the picture to be reproduced, is supplied with prepared color offering a sufficient resistance to the etching or dissolving medium, and one or preferably 25 several exactly registering impressions are made, first on one side and then on the other of the prepared paper sheet having on both sides the etchable coating.

The printed sheet of prepared paper is 30 then subjected for a short time to the action of an etching agent to destroy the binding qualities of the adhesive in the etchable coating, where exposed to the action of such agent, and the coating, where the adhesive 35 agent is so destroyed, is removed by washing or brushing, so that a relief is obtained corresponding to the picture.

It is thus possible to obtain, by the use of 40 a paper coated with an etchable material of this character, strong relief values accurately graduated in all details, and the height of the relief may be exactly regulated by the thickness of the coating and by the 45 duration of the etching process.

Surfaces of the same tone are thus always 50 of the same height, and when so produced, may be used as an overlay on the printing cylinder or platen, or as an underlay between the printing form and the support.

Having thus fully described the nature

of my invention, what I claim as new and desire to secure by Letters Patent, is:—

1. In the herein described article of manufacture, a sheet of paper having an etchable coating comprising blanc fixe, china 55 clay, aluminum acetate, and an adhesive.

2. In the herein described article of manufacture, a sheet of paper having an etchable coating comprising blanc fixe, china clay, an agent to aid the etching qualities 60 of the coating, and an adhesive.

3. In the herein described article of manufacture, a sheet of paper having an etchable coating comprising blanc fixe, china clay, glycerin, aluminum acetate, and an ad- 65hesive.

4. In the herein described article of manufacture, a sheet of paper having an etchable coating consisting of blanc fixe, china clay, glue, glycerin and aluminum acetate, 70 in the proportion of two hundred and ninety pounds of blanc fixe, five hundred and eighty pounds of china clay, one hundred and twenty-five pounds of glue, two pounds of glycerin, and twelve ounces of aluminum 75 acetate.

5. In the herein described article of manufacture, a sheet of paper having an etchable coating comprising a mineral body and aluminum acetate.

6. In the herein described article of manufacture, a sheet of paper having an etchable coating comprising a mineral body, aluminum acetate, and an adhesive.

7. In the herein described article of manufacture, a sheet of paper having an etchable coating comprising a mineral body, and an agent to aid the etching qualities of the 85 coating.

8. In the herein described article of manufacture, a sheet of paper having an etchable coating comprising a mineral body, an agent to aid the etching qualities of the coat, and an adhesive.

Toronto, September 22nd, 1917.

JAMES MILN.

Signed in the presence of

CHAS. H. RICHES,  
EDWARD D. BERNSTEIN.